

# UNITED STATES PATENT OFFICE.

BENJAMIN TALBOT, OF DARLINGTON, ENGLAND.

## PROCESS OF MAKING STEEL AND INGOT-IRON.

985,225.

No Drawing.

Specification of Letters Patent. Patented Feb. 28, 1911.

Application filed April 4, 1910. Serial No. 553,260.

To all whom it may concern:

Be it known that I, BENJAMIN TALBOT, a British subject, residing at Woodburn, Darlington, county of Durham, England, have 5 invented an Improved Process of Making Steel and Ingot-Iron.

My invention is an improvement on the Bessemer and continuous processes of manufacturing steel and ingot iron.

10 It consists in subjecting unrefined molten metal, taken from a blast furnace, cupola or mixer, to a surface blast, or blast through the upper strata of the metal, by which the bulk of the silicon and a greater or less percentage of other metalloids are eliminated, 15 with conversion of graphite into combined carbon, and the production of an oxidizing slag; then pouring further metal to be refined through the slag of the metal blown 20 and blowing the combined charges to effect the desired oxidation of the contained metalloids, the metal being preferably transferred for final oxidation to a finishing furnace.

25 In practice, a basic lined converter having a capacity of fifty to one hundred tons is preferably employed and an initial charge is introduced of say half the converter's capacity. This metal is subjected to surface 30 blast or a blast directed through its upper strata, which produces considerable oxid of iron slag and agitates the metal, with the elimination of the bulk of the silicon and more or less of the remaining metalloids, 35 and changes to the combined form the bulk of the graphitic carbon not eliminated, the latter change avoiding the foaming and occasional explosions taking place in the treatment of liquid metal containing graphitic 40 carbon in finishing furnaces. The initial charge having been thus treated, the further half of the metal is poured through the slag, effecting a precipitation and recovery of iron from the iron oxid in the slag and the 45 oxidation of the metalloids of the added iron. The full charge is now blown until the impurities are eliminated to the extent desired, when a part or all of the metal is tapped in a condition considerably hotter 50 than is usual.

The blowing is effected at a comparatively short distance below the surface of the metal and consequently a low pressure suffices for the introduction of the blast.

55 Preferably part of the metal is tapped

from the converter and the remainder is left for admixture with a further charge of impure metal to be treated.

The practice of the process may be illustrated by its application to the treatment of say fifty tons of molten metal containing 60 3.7% carbon, 1.25% silicon and .8% manganese. Of this metal about twenty-five tons are run from the blast furnace, mixer or cupola into the converter and subjected to 65 a surface blast, or blast through its upper strata, until the silicon has been oxidized down to say .25% or under, the manganese to say .5% or even traces, and the carbon to say  $\frac{1}{2}$  or  $\frac{1}{3}$  the original content, the graphitic 70 carbon which may have been 1% having been reduced to the combined form. The above conditions having been attained, the remainder of the charge, consisting of about twenty-five tons of impure metal, is run 75 into the bath. More or less reaction takes place and the combined metal is blown until the silicon has been reduced to .25% or less, the manganese to .5% or even traces, and the carbon to about 2.75% or under, the remaining carbon being practically all in the 80 combined form, which is of great advantage in the further treatment in the finishing furnace. All or part of the metal in this condition is now tapped and run into the 85 finishing furnace which is advantageously of the continuous open hearth type, though an electric or other form of finishing furnace may be employed.

Having described my invention, I claim: 90

1. The process of manufacturing iron and steel which consists in subjecting a charge of unrefined molten metal to a surface blast and producing an oxid of iron slag, adding a further charge of metal to be purified, and 95 blowing the combined charges.

2. The process of manufacturing iron and steel which consists in blowing the upper strata of a charge of molten metal, producing thereby an oxid of iron slag, eliminating the bulk of the silicon, eliminating part of the carbon and converting the bulk of the remaining graphitic to combined carbon, then adding further impure metal and blowing the combined charges. 100

3. The process of manufacturing iron and steel which consists in placing a charge of unrefined metal in a converter, subjecting said metal to surface blowing so as to produce an oxidizing slag and eliminate the 110

2  
bulk of the silicon with more or less of the  
other metalloids, adding a further charge of  
unrefined metal to the bath and blowing the  
combined charges, tapping metal from the  
5 converter and subjecting it to further treat-  
ment in a finishing furnace.

In witness whereof I have hereunto set

my name this 2nd day of April, 1910, in the  
presence of the subscribing witnesses.

BENJAMIN TALBOT.

Witnesses:

ROBERT JAMES EARLEY,

Jos. G. DENNY, Jr.